

Patented May 16, 1933

1,909,916

# UNITED STATES PATENT OFFICE

ORA S. DUFFENDACK AND RALPH A. WOLFE, OF ANN ARBOR, MICHIGAN

ELECTRON EMITTER AND METHOD OF MAKING SAME

No Drawing.

Application filed May 11, 1931. Serial No. 536,676.

This invention has to do with electron emitting elements and the process of making them. Such elements are used in vacuum tubes of various kinds, for example, those employed as rectifiers, detectors, amplifiers and the like to produce a desired electronic flow. The elements will also find use in low pressure gas filled tubes used for low voltage rectification, such as the well known Pliotron tubes. Another field of use for our emitting element is in the luminous gas tubes, lamps, and the like such as the well known Neon sign lamps, air-way beacon lights and the like.

The electron emitter heretofore employed in such vacuum tube devices have usually consisted of a suitable base metal, such as nickel, tungsten, platinum, copper, or in some cases, special alloys, such as the Konel alloy, provided with a coating of oxides of one or more of the alkaline earth metals, usually the oxides of barium or strontium. The base metal gives the desired mechanical strength to the filament, resisting deformation at the temperatures at which it is used, while the coating gives the desired high rate of electron flow.

In the preparation of such elements for use in the tubes it has been common practice to first thoroughly clean the base metal, then oxidize it and spray or otherwise deposit upon it a coating of the oxides or carbonates. This coating is allowed to dry, and the element is then ready for insertion in the tube. Then follow the customary steps of exhausting the tube in various stages and heating the parts of the tube and flashing the getter to remove all possible traces of gas. The tube is then sealed, and the next step is activation. This usually consists in heating the emitter to a suitable temperature, usually around 800° C., for a sufficient length of time to produce the desired or maximum rate of emission. An emitter manufactured by this, or similar methods, consists essentially of a

base metal with an applied oxide coating adhering closely to it. The relatively high emissivity results from the pressure in the coating of free metallic barium obtained by breaking down, or reducing, the oxide of the coating. While such emitters have been the best produced prior to our invention, they have been subject to the following objections:

1. It has proven very difficult to cause the coating to firmly adhere to the base metal, and many tubes are rejected upon final inspection because the coating has flaked off.

2. It has been found difficult to produce tubes of the same electron emission under the same conditions in the process of manufacture for mysterious unknown reasons. Often times tubes manufactured under exactly similar conditions as before, will have a very marked decrease in electron emission. This makes it impossible to obtain uniform results even with identically the same apparatus in the case of radio receivers, and the like.

3. It has been practically impossible to secure a coating of uniform thickness on the base metal, and this results in hot spots where the coating is uneven. The hot spot causes the coating to flake off, or, in some cases, results in the burning out of the filament.

4. The rate of emission from coated filaments is quite variable increasing at first and then decreasing from the maximum with the increase in the usage of the tube. The requirement of initial electronic emission higher than necessary to insure adequate emission over extended periods of use makes it necessary to reject many tubes upon final inspection.

5. There is a wide variation in the length of time that a tube made with an oxide coated emitter is serviceable or usable.

6. We have indicated above some of the objections to oxide coated emitters, and it should now be clear that the processes used in their manufacture are attended with many

difficulties and with considerable loss in imperfect tubes. The variable character of the coating, and the fact that it is readily attacked by moisture, and carbon-dioxide before being assembled into the tube further aggravates the situation.

7. There is also a class of emitters consisting of tungsten, tantalum, or molybdenum. In the case of tungsten these pure metallic emitters have been improved by rolling thorium oxide into the base metal, or otherwise combining them. While such emitters are free from most of the objections to the coated emitter, as pointed out above, they are 10 unsatisfactory in that they must be heated to high temperatures to get the desired amount of emission, and as a consequence their efficiency is low. In the case of the 15 thoriated tungsten emitter, if it is accidentally subjected to high temperatures the thorium may be entirely driven off, rendering the tube useless.

Our invention consists in a new type of 20 emitter which is free from applied coatings with their attendant disadvantages, and which at the same time yields in usual operation a high rate of electron emission at a 25 relatively low temperature, the rate of emission remaining substantially unchanged over 30 long periods of use. Our emitter is also characterized by uniformity, it being possible to duplicate tubes to a degree not possible heretofore in low temperature emitters. Our 35 emitters are produced by a method which is very simple and readily adapted to manufacture. The employment of our method and the emitter which results from it will also reduce, to a very considerable degree, the cost 40 of manufacture, and will practically eliminate the large number of rejections now resulting from faulty emitters.

Our emitter consists of an alloy of a base 45 material and material having a high rate of electronic emission. A very important difference between our emitter and those of the prior art resides in the fact that the base material not only gives the emitter the necessary stiffness, but also, when treated by our process, prevents evaporation from the surface of the emitter, and assists in holding upon it the active emitting material. The base material, when so treated, is likewise responsible for a large increase in thermionic 50 emission.

55 For the base material we may use nickel, or preferably an alloy of nickel and chromium. To the nickel or nickel alloy may be added a small amount of manganese or calcium to render the alloy easier to roll and draw. For the material of high electron emissivity we may employ the alkaline earth metals barium, strontium or calcium, either alone, or in combination with each other, or with thorium, or other well known active 60 materials. It will be noted that the active 65

materials are electropositive with respect to the base metals.

|                | Per cent  |
|----------------|-----------|
| Barium         | .01 to .2 |
| Manganese      | 1½ to 2   |
| Chromium       | .5 to 10  |
| Balance nickel |           |

We give below an example of an alloy falling within the above range with which we 75 have had particular success:

|                | Per cent |
|----------------|----------|
| Manganese      | 1½ to 2  |
| Chromium       | 2        |
| Barium         | .15      |
| Balance nickel | 80       |

The ranges of ingredients given above are suggestive rather than limiting. Thus the percentage of barium given extends from the lowest amount that will be found to be of any practical use in electron emitting devices. 85 We have in mind particularly the rather feeble emitter used in telephony. The emission rapidly increases with the amount of 90 barium in the alloy.

The range of percentage of chromium is determined from the change in the thermionic emission with the change in the percentage of chromium, the other ingredients 95 remaining constant in amount. Beneficial effects from the addition of chromium were observed at .5% chromium. The benefits increased until the maximum thermionic emission was reached at 3% chromium; after 100 which the thermionic emission again decreased until at 10% very little advantage from the addition of chromium was observed. At percentages of chromium above 10% the rate of evaporation of the alloy became 105 excessive at the temperatures at which the emitters were maintained. The use of molybdenum, tungsten or uranium in place of chromium is indicated because of the similar properties of these elements.

110 The amount of manganese specified is simply that customarily used to deoxidize the nickel and render the alloy easier to roll and draw. There may, of course, be the usual variation in the percentage of this material 115 in the alloy. The manganese, we have found, has very little, if any, effect on electronic emission, and it is added primarily for convenience in manufacture. Other known materials such as calcium may be used for this 120 purpose.

The alloys may be formed by the method claimed in the prior application of Donald W. Randolph, Serial No. 520,704, filed March 6, 1931.

125 We have also made up alloys in which, in addition to the barium, we have included strontium, calcium, thorium, or a combination of these metals.

130 With the alloy, as described, drawn into wires, or formed into other shapes that may

be desired, we are ready for the next step. We have found that by means of a suitable heat treatment the above mentioned alloys can be put into such condition (activated)

5 that they will emit electrons at a much higher rate. In actual practice we have found that the use of this process results in increasing the emission from the alloy about one hundred (100) times. This heat treatment also 10 results in placing the alloy surface in such condition that the emission is maintained very uniformly over long periods of use.

The activation process is divided into two parts, the first of which consists in heating 15 or oxidizing the surface of the alloy in air preferably at atmospheric pressure. In order to produce the maximum electron emission, the wire must be heated so as to form an oxide film. This film in the case of the 20 nickel, barium chromium manganese alloy is of a dark blue color having in it a greenish tint due to the chromium oxides. We have found that this preliminary heating in air may be carried out at temperatures from 25 350° C. to 800° C. The time during which the wire must be held at any temperature depends on the temperature selected. At 350° C. it is necessary to heat the wire for approximately one-half hour to produce a sufficient 30 surface oxidation. At 600° C., satisfactory oxidation can be produced in 30 seconds; at 700° C. in five seconds; at 800° C. in two seconds. The lower temperature limit of 350° C. is possibly not the lowest temperature at which 35 the surface can be oxidized, but on account of the time required at this or lower temperatures, the temperature of 350° C. is considered the lowest practicable temperature. The upper limit of temperature at which the 40 oxidation process may be carried out is the melting point of the alloy, it being understood that as the temperature is increased the time must be decreased. If too high a temperature or too long a time is used, the efficiency of the emitter is decreased rather than increased, while if too low a temperature is used, or the time is too short the full benefits of this oxidation process are not realized.

The preferred temperature range for oxidation is, from our present experience, from 50 700° to 750° C. at which temperatures the wire must be held for a time ranging from 5 to 3 seconds.

If air pressures less than atmospheric are 55 used, the oxidation of the surface is retarded and either the time or the temperature must be increased as the pressure is decreased. It must be understood that if the oxidation be carried out in a chamber at reduced pressures, the amount of oxygen in the chamber must be sufficient to produce the required degree of oxidation of the surface.

If the oxidation is carried out in an atmosphere of pure oxygen instead of air, the time 60 required for the oxidation process at any

given temperature is less than when the surface is oxidized in air alone. We have found that the oxidation process may be carried out slowly in an atmosphere of CO<sub>2</sub> and this indicates that possibly other gases might be employed although time and temperature relations for these gases would of necessity be different.

We wish to emphasize the fact that the degree of oxidation of the surface is not so critical but that a considerable tolerance of time and temperature may be permitted. The amount of oxidation produced by heating the wire in air at 700° C. for 5 seconds is such that the rate of activation of the emitter when assembled in a vacuum tube is convenient and practicable. If the degree of oxidation is materially greater than this, the rate of activation is decreased to such an extent as to make the emitter less practicable for commercial use.

Even within the considerable range of oxidation treatment as disclosed above, subsequent additional activation is realized in the 70 second step of the process.

The second step in the method used for producing an active specimen of the alloy consists in assembling a filament made of the alloy in a vacuum tube and heating it in a good vacuum to a temperature of 1150° C. for a period of from 15 minutes to one hour, then reducing this temperature to approximately 1000° C. until the thermionic emission has reached the desired stabilized value. If an initial heating temperature lower than 1150° C. is employed, the specimen must be maintained at that temperature for a longer period of time to insure complete activation of the surface. We have found that the increase in thermionic emission is more rapid and that it reaches a greater value if no electron current is drawn from the emitter during the activation period. During the activation process, barium diffuses from the interior of the wire to the surface where it is securely held by the oxide film.

It would appear as though the presence of oxides of nickel and/or chromium, as formed in the first step of this process, is necessary to obtain a large increase in thermionic emission over similar alloys not so treated. We have demonstrated that the oxide surface prevents the rapid evaporation of the active emitting element. We have also evidence that the oxide surface reduces the rate of evaporation of the alloy as a whole,—that is, the metals of the alloy. This fact would probably reduce the rate of evaporation of the active oxide by preventing its being carried off by the evaporating metals. Whatever be the correct explanation of the phenomena, the oxide surface apparently prevents evaporation from the electrode surface and assists in holding upon it the barium that has been 120 125 130

caused to diffuse to this surface by the second step of the process.

We have secured the best results from this method of treatment by employing the above alloy containing chromium. However, for some purposes satisfactory results may be obtained without the use of chromium. Such an alloy may be in the following proportions:

|                   | Per cent  |
|-------------------|-----------|
| 10 Barium         | .01 to .2 |
| 15 Manganese      | 1½ to 2   |
| 20 Balance nickel |           |

This alloy may be treated in the manner previously described, and we have found the time and temperature treatment to secure maximum results is substantially the same. This alloy is not as satisfactory as the chromium alloy for the reason that the electron flow is smaller and the rate of evaporation of barium from the surface is greater. It has also been observed that the rate of evaporation of the alloy itself is greater when it contains no chromium. Furthermore, it is possible to maintain the chromium alloy at a higher temperature without deactivating the emitter than is the case with the alloy without chromium.

It is obvious that the emitter may take any form that may be desired, and that convenience in manufacture may dictate such expedients as oxidizing the emitter in the vacuum tube rather than previous to its insertion. Our emitters when operated at the usual temperatures to which oxide coated filaments are now subjected will give a rate of emission of the same order of magnitude as the oxide coated emitters without showing any practical difference in emissivity from one tube to the next. The method of manufacture is obviously simple and easy. We have tested our emitters over long periods of time, and find that at the ordinary operating temperature the saturation emission current shows no decrease over the period of the test whereas it is well known that the saturation emission current of an oxide coated emitter will fall off at a considerable rate.

We may use in place of the barium in the above described alloys any one or more of the other alkaline earth metals, such as strontium, or calcium. The alloys thus formed may be oxidized and activated in the manner described. However, for best results, we prefer the barium containing alloys.

We have described the activating step as heating the emitter in vacuum. The activation, of course, may be effected by heating the emitter in an atmosphere of inert gases, such as argon, helium and so forth. Whether the activation is accomplished in vacuum, or whether in an atmosphere of inert gases, we have included it in the descriptive phrase "activated in a non-oxidizing atmosphere."

The heating in the activation process may be accomplished in any manner, whether by heat conduction, or electrical conduction, or by inductive effect.

We claim:

1. The process of producing an electron emitter which consists in preparing an alloy consisting chiefly of a base metal with a small proportion of a metal of high electron emissivity, oxidizing the alloy to produce a surface composed of oxides of the emitting metal and of the base material, and thereafter heating the emitter, the oxides of the base metal and of the emitting metal preventing the rapid evaporation of the material of high electron emissivity. 70
2. Process of producing an electron emitter which consists in preparing an alloy consisting chiefly of malleable nickel with a small proportion of an alkaline earth metal to impart high electron emissivity thereto, oxidizing the alloy to produce a surface composed of the oxides of said metals and activating the alloy by heating it in a non-oxidizing atmosphere. 80
3. The process of producing an electron emitter which consists in preparing an alloy consisting chiefly of a base metal and small proportions of chromium, and a metal of high electron emissivity, oxidizing the alloy to produce a surface composed of the oxides of said metals and activating the alloy by heating it in a non-oxidizing atmosphere. 90
4. A process of producing an electron emitter which consists in preparing an alloy consisting chiefly of nickel including small proportions of chromium, and an alkaline earth metal, oxidizing the alloy to produce a surface composed of the oxides of said metals and heating the alloy, the oxidized surface serving to retain the material of high emissivity. 100
5. The process of producing an electron emitter which consists in preparing an alloy consisting chiefly of malleable nickel including small proportions of chromium and barium, oxidizing the alloy to produce a surface composed of the oxides of said metals, and subsequently heating the emitter formed therefrom, the oxidized surface preventing rapid evaporation of the metal of high emissivity. 110
6. An electron emitter formed of an alloy of a base metal and a metal of high electron emissivity having a coating of the oxides of said metals. 120
7. An electron emitter formed of an alloy of a base metal, including chromium and a metal of high electron emissivity, said emitter having a coating of the oxides of said metals. 125
8. An electron emitter formed of an alloy of nickel and an alkaline earth metal and having a coating of the oxides of said metals. 130

9. An electron emitter formed of an alloy of nickel and barium having a coating of the oxides of said metals.
10. An electron emitter formed of an alloy of nickel, chromium and barium and having a coating of the oxides of said metals.
11. An electron emitter formed of an alloy of nickel, chromium and barium and having a coating of the oxides of said metals, and metallic barium.
12. An electron emitter formed of an alloy of malleable nickel, chromium and barium having a coating of the oxides of said metals.
13. The process of producing an electron emitter which consists in forming an emitter of an alloy consisting chiefly of nickel and barium, oxidizing the alloy by heating it in air to a temperature not substantially less than 350° C. and thereafter heating the alloy in a non-oxidizing atmosphere to a temperature upward of 1000° C. to produce an activated surface.
14. The process of producing an electron emitter which consists in forming an emitter of an alloy consisting chiefly of nickel with lesser amounts of chromium and barium, oxidizing the alloy by heating it in air to a temperature not substantially less than 350° C. thereafter heating the alloy in a non-oxidizing atmosphere to a temperature upward of 1000° C. without drawing current therefrom, and continuing said heating until a highly activated surface is obtained.

In testimony whereof we affix our signatures.

ORA S. DUFFENDACK.  
RALPH A. WOLFE.

40

45

50

55

60

65